

1,359,719.

G. A. MEAD.

METHOD OF MAKING COMPOUND METALLIC ARTICLES.  
APPLICATION FILED OCT. 22, 1919.

Patented Nov. 23, 1920.



Fig. 1



Fig. 2



Fig. 4



Fig. 3



Fig. 5



Fig. 6

Inventor

Witness

*D. S. Mathews*

By

*George A. Mead*

Attorney

# UNITED STATES PATENT OFFICE.

GEORGE A. MEAD, OF MANSFIELD, OHIO, ASSIGNOR TO THE OHIO BRASS COMPANY, OF MANSFIELD, OHIO, A CORPORATION OF NEW JERSEY.

## METHOD OF MAKING COMPOUND METALLIC ARTICLES.

1,359,719.

Specification of Letters Patent. Patented Nov. 23, 1920.

Application filed October 22, 1919. Serial No. 332,459.

To all whom it may concern:

Be it known that I, GEORGE A. MEAD, a citizen of the United States of America, residing at Mansfield, in the county of Rich- 5 land and State of Ohio, have invented cer- tain new and useful Improvements in Meth- ods of Making Compound Metallic Articles, of which the following is a specification.

My invention relates to the process of uniting bodies of unlike metals and especially to processes in which the unlike metals are so firmly united by a weld as to resist the action of both temperature changes and mechanical stresses and whereby a union of high elec- 5 trical conductivity is attained.

My invention is of particular value in uniting such metals as iron or steel with copper or copper alloys although it is applicable to the uniting of other dissimilar 10 metals.

It is also of value where it is desired to unite to steel or iron a mass of copper or copper alloy which is of intricate shape and such as can be produced only to advantage 15 by means of molds. A process of this character has particular value in producing various electrical devices in which intricate shapes of a high conducting metal are to be united to steel or iron and in which the union 20 must be practically that of a weld and I will describe the application of my invention to such metals although it is applicable to others.

In the drawing which illustrates my in- 25 vention:—

Figure 1 shows a steel or iron bar which may be of various shapes or sections.

Fig. 2 shows the application thereto of a metallic coating which is to form an insepa- 30 rable union with the bar and have a melting point lower than that of the copper or copper alloy to be united to the bar.

Fig. 3 shows a modified method of applying a metallic coating to the steel or iron 35 bar.

Fig. 4 shows the application of the copper or copper alloy member to the bar which has been prepared as shown in Fig. 2 or 3.

Fig. 5 shows the steel or iron bar and the 40 copper or copper alloy mass as united by my process.

Fig. 6 shows a part section of the article in Fig. 5 and represents the intimate union between the bar and copper or alloy mass.

In carrying out my invention I take a 55 bar 1 as shown in Fig. 1 of suitable size and shape and which may be of rolled or cast metal and of steel or iron. To this bar I apply to the surface thereof a coating 2 of a metal which has the property of strongly 60 uniting or alloying with the steel and forming an inseparable union therewith except as the same may be removed by melting, acid, grinding, or filing, etc. This coating may be composed of copper and zinc forming the 65 ordinary brazing metal of about sixty percent copper and forty percent zinc and is preferably of a lower melting point than that of the copper or copper alloy applied thereto but which will readily alloy there- 70 with. The coating may be of pure copper or a copper-tin alloy or other metals which will meet the requirements as herein set forth.

In applying the coating I have found that 75 this can be most readily performed by means of the oxyacetylene flame 3 or other high temperature flames, that of oxyacetylene being about 6400 degrees Fahrenheit. In applying the coating by a high temperature flame the coating forms a union which is permanent as it is to all intents and purposes alloyed to the steel or iron member. The application of the coating is made by 80 heating small areas of the surface of the bar and melting unto such heated areas the coating metal 2 which is supplied in the form of rods or sticks 4 and progressively extend 85 this process of treating small areas until the desired surface of the bar has received a 90 proper coating. It will be understood that a suitable fluxing agent may be used on the surface of the steel if desired and such fluxing agent may be powdered borax which is melted or fused on the surface of the bar before 95 applying the coating metal. I have found, however, that by applying the coating metal with the oxyacetylene or other high tempera- 100 ture flame that it is not necessary to use a fluxing agent although there are at times 105 advantages in so doing.

A modified method of applying the coating is shown in Fig. 3 and consists in melting in a refractory pot 5 or other suitable container the metal 6 to be used as a coating. To 105 prevent rapid oxidation of this coating metal and to assist in the union of the coating metal 6 to the rod 1, the top of the coating

metal may be covered with a fluxing material 7 such as borax, potassium chlorid, etc. The bar 1 is first heated and a fluxing agent such as borax applied to that part to be coated 5 and fused thereon and such treated surface is then plunged through the flux 7 into the molten coating metal.

It will be found of advantage to have the 10 temperature of the bar 1 equal to or slightly greater than that of the coating metal 6, thereby securing a smoother, thinner and more adhering coating.

After preparing the iron or steel bar 1 with the coating metal 2 the bar is ready to 15 have applied thereto the copper or bronze portion and if this is of such shape as to require forming in a mold, the bar 1 is properly embedded in the sand 8 as shown in Fig. 4 with the coated surface extending into the 20 mold cavity 9. The molten copper or bronze 10 which is to fill the cavity 9 and form a part of the bar 1 when solidified, is now poured into the mold and preferably allowed to flow over the coating on the rod thereby 25 heating the rod and the coating and causing the coating and molten copper or bronze to form an alloy, the one with the other and, whereby a practically one-piece article is produced in which the copper or bronze 30 member 11 and rod 1 are inseparably united by a union which is practically the equal of a perfect weld.

Upon sectioning and examining the union 35 between the bar 1 and the copper or bronze member 11 it will be found that the two have formed an inseparable union through the medium of the coating metal and which has to a large degree lost its identity by 40 alloying with the member 11 and a careful study of the union produced by my method will show no definite line of demarcation 45 between the bar 1 and the member 11.

In applying the coating with the oxyacetylene or other high temperature flame the 45 surface of the bar 1 is brought to the point of fusion and when the coating metal is melted on to such fused surface it immediately alloys therewith and the molten copper or bronze 10, having a higher melting 50 point than that of the coating metal, will, when properly applied thereto, cause the coating metal to melt and an alloy is formed between the two.

What I claim as new and desire to secure 55 by United States Letters Patent is:—

1. The process of making an article of two dissimilar metals comprising the steps of applying to the surface of one of the metals a dissimilar coating metal of a lower 60 melting point to act as a nexus by fusing the surface of one of the dissimilar metals, then fusing the coating metal and applying it to the fused surface of the one metal, then fusing the metal to form the second 65 dissimilar metal referred to and then ap-

plying it while fused to the coating metal and at a higher temperature than the melting point of the coating metal.

2. The process of making an article of manufacture composed of dissimilar metals 70 comprising the steps of coating the surface of one of the metals with an alloy composed of copper and zinc, then applying to the coating the other dissimilar metal in a molten condition and at a temperature 75 higher than the melting point of the coating metal.

3. The process of making an article of manufacture of dissimilar metals comprising the steps of fusing the surface of one 80 of the metals, then applying thereto in a fused state a dissimilar metal, comprising an alloy having a copper base and of a lower melting point than the metal to which it is applied to form a coating, then 85 inserting the metal with the coating in a mold formed with a cavity, then applying to the coated surface a stream of molten metal having a higher melting point than that of the coating and filling the cavity 90 therewith.

4. The process of making an article of manufacture composed of dissimilar metals comprising the steps of fusing the surface of one of the metals, then applying to the 95 fused surface a coating of a copper base alloy, then applying to the coating the other dissimilar metal in a molten condition and at a temperature higher than the melting point of the coating metal.

5. The process of making an article of manufacture composed of two dissimilar metals of different melting points comprising the steps of fusing a small surface area of the metal having the higher melting 105 point, then melting on and alloying to this surface while still fused a metallic coating, then repeating this operation of fusing and covering until the desired area has been treated, then applying to the coating the 110 second dissimilar metal, of a higher melting point than the coating metal and dissimilar thereto, in a molten condition and at a temperature higher than the melting point of the coating metal and then allowing the 115 second dissimilar metal to solidify.

6. The process of making an article of manufacture composed of two dissimilar metals of different melting points comprising the steps of fusing a small surface area 120 of the metal having the higher melting point, then melting on and alloying to this surface while still fused a metallic coating having a lower melting point than the two dissimilar metals and dissimilar to each, then repeating this operation of fusing and covering until the desired area has been treated, then applying to the coating the 125 second dissimilar metal in a molten condition and at a higher temperature than the 130

melting point of the coating metal and then allowing the second dissimilar metal to solidify.

7. The process of making an article of manufacture composed of two dissimilar metals of different melting points comprising the steps of first applying a heating flame to a small area of the surface of the metal having the higher melting point to 5 alloyed coating, then repeating this operation of fusing and covering until the desired area has been treated, then applying to the 15 coating the second dissimilar metal of a higher melting point than the coating metal, in a molten condition and at a temperature higher than the melting point of the coating metal and then allowing the second dissimilar metal to solidify. 20
- 10 fuse said localized area, then fusing and applying to said small area and by said same heating flame a metal to form an

In testimony whereof I affix my signature.

GEORGE A. MEAD.